

**[54] TANTALUM CARBIDE-TANTALUM FIBER COMPOSITE MATERIAL****[75] Inventors:** Robert E. Riley; James M. Taub, both of Los Alamos, N. Mex.**[73] Assignee:** The United States of America as represented by the United States Atomic Energy Commission, Washington, D.C.**[22] Filed:** Jan. 18, 1972**[21] Appl. No.:** 218,686**[52] U.S. Cl.:** 29/182.8, 75/204, 75/DIG. 1**[51] Int. Cl.:** C22c 29/00**[58] Field of Search:** 75/DIG. 1, 203, 204; 29/182.7, 182.8**[56] References Cited****UNITED STATES PATENTS**

3,285,825 11/1966 Jens ..... 75/DIG. 1

|           |         |                       |           |
|-----------|---------|-----------------------|-----------|
| 3,149,253 | 9/1964  | Luebke .....          | 75/DIG. 1 |
| 3,479,155 | 11/1969 | Rudy .....            | 29/182.7  |
| 3,114,197 | 12/1963 | De Bois et al. ....   | 75/DIG. 1 |
| 3,352,650 | 11/1967 | Goldstein et al. .... | 75/DIG. 1 |

*Primary Examiner*—Carl D. Quarforth*Assistant Examiner*—E. A. Miller*Attorney*—John A. Horan**[57] ABSTRACT**

The thermal stress resistance of refractory metal carbides is substantially improved by the addition of chopped metal fibers. A composite consisting of 50 vol percent TaC-50 vol percent chopped Ta wire shows approximately a 40 percent improvement in thermal stress resistance over that of pure TaC.

**1 Claim, 1 Drawing Figure**

ATENTED DEC 18 1973

3,779,716



## TANTALUM CARBIDE-TANTALUM FIBER COMPOSITE MATERIAL

### BACKGROUND OF THE INVENTION

The invention described herein was made in the course of, or under, a contract with the U. S. ATOMIC ENERGY COMMISSION. It relates to structural materials having improved thermal stress resistance at temperatures in excess of 2,000° C and more particularly to such materials consisting of refractory metal carbide-refractory metal fiber composites.

It is known in the art that structural materials exposed to temperatures in excess of 2,500° C for any substantial period of time, i.e., for more than 60 minutes, rapidly degrade. Refractory metal carbides are obvious candidates for such structural materials. However, they are brittle and readily crack in such temperature regimes. This cracking in turn rapidly leads to complete fracturing which may result in a catastrophic failure of the particular structure. As used within this application, fracturing means the separation of a massive body into two or more smaller bodies.

### SUMMARY OF THE INVENTION

We have now found that the addition of a chopped metal fiber to the refractory metal carbide will substantially enhance the thermal stress resistance of the carbide. The refractory metal carbide-metal fiber composites may readily be formed through hot pressing. While various refractory metal carbides may be used as the matrix material, it is desirable that the carbide be a mono- rather than a dicarbide. Various chopped metal fibers such as Ta, Mo, 75 vol percent W-25 vol percent Re, Re, etc., may be used. In particular, chopped rhenium fibers are useful because rhenium does not form a carbide. The limiting factor in the use of a particular metal fiber in the composites of this invention is the formation of the metal carbide-carbon eutectic. It will be apparent that the use of a metal fiber M as a reinforcing material in a metal carbide matrix is undesirable if the temperature of the MC-C eutectic is below that to which the composite will be exposed in its structural use. In the case of rhenium, the limiting temperature regime is that at which the Re-C eutectic occurs. The temperatures at which the various refractory metal carbides form eutectics with carbon are well known in the art.

We have found that a composite consisting of 50 vol percent TaC-50 vol percent chopped Ta wire shows approximately a 40 percent improvement in thermal stress resistance over that of pure TaC. At temperatures in excess of 2,500° C, a composite material of this type will still crack, but the presence of the fibers inhibits the propagation of the cracks completely through the structure so that fracturing is avoided or substantially reduced. As can be seen from the FIGURE, up to about 70 vol percent Ta, TaC-chopped Ta wire composite materials exhibit isotropic thermal characteristics. This indicates that neither the size nor the diameter to length ratio of the chopped metal fibers is critical in the composites of this invention. Indeed, it suggests that the metal need not be present as fibers at all but may serve as well in an irregular particulate form.

### BRIEF DESCRIPTION OF THE DRAWING

The FIGURE compares the results of steady-state thermal stress testing of various TaC-chopped Ta wire

specimens machined in both the parallel and perpendicular to the pressing direction with that of a pure TaC specimen tested in the parallel direction only.

### DESCRIPTION OF THE PREFERRED EMBODIMENT

Tantalum wire 20 mils in diameter was chopped to approximately 0.25 inch lengths and blended in desired proportions with TaC powder having 1.5 micron nominal size. The blended material was then hot pressed at 1,800° C for a time sufficient to produce a density of about 80 to 85 percent theoretical. Typically, this took about one-half hour.

Steady-state thermal stress specimens were machined from the 10, 50, 60, and 70 vol percent Ta wire billets in both the parallel and perpendicular to the pressing direction. The FIGURE compares the results of steady-state thermal stress testing on these materials with that of pure TaC specimen tested in the parallel direction only. The 100 percent TaC material was ~ 96 percent of theoretical density. There is clearly a significant increase in thermal stress resistance associated with certain contents of Ta fiber. With the exception of the 30 vol percent TaC-70 vol percent specimens, the material is isotropic. Whereas pure refractory metal carbides have steady-state thermal stress resistances in the range of 500° to 650° C radiator temperature, the 50 vol percent TaC-50 vol percent chopped Ta wire composite material has a steady thermal stress resistance at about 900° C radiator temperature. This is an improvement of about 40 percent over that of TaC alone.

One-inch-o.d. by one-quarter-inch-i.d. by one-sixteenth-inch-thick specimens of TaC reinforced with 60 and 70 vol percent chopped Ta wire were thermally shock tested. There was a large difference in the power setting required to initiate a crack and the power setting required to completely fracture the materials. Typically, a crack could be made to initiate at a power setting of ~ 80-110 and then to propagate (sometimes across the entire specimen). However, these cracks were very tight and did not significantly degrade the strength of the specimen. Apparently the Ta wires bridging the cracks act in effect as tiny reinforcing bars. With the thermal shock instrumentation used, pure refractory metal carbides require power settings of 60 to 80 for crack initiation. In such carbides, however, only a slight increase in the power setting leads to rapid fracture.

It was only at power settings in excess of 200 that these materials could be fractured. In fact, the with-grain specimens could not be fractured at all, even though, at these power settings, the specimens had so many cracks that they resembled cracked safety glass. Several specimens were finally forced to part into two pieces by melting the Ta wires holding the cracked segments together.

The thermal shock data for these materials are summarized in Table I. As can be seen, two thermal shock indices are given; one pertains to crack initiation and one pertains to fracture. This latter index is more important in terms of the ultimate capability of these materials. Included in Table I for comparison are the results for with-grain RVC graphite. As can be seen, crack initiation was not obtained with RVC; rather fractures through the washer occur.

Room temperature comparative thermal conductivity data were also obtained on these materials. Table II

presents a comparison between the experimental and predicted values of the thermal conductivity. The model assumed is a dispersion of Ta wires in a continuous matrix of TaC. The axes of the wires are assumed to be parallel to the radial plane of the pressing, but randomly oriented in that plane. The porosity relationships were those derived for hot-pressed ZrC.

Table I  
THERMAL SHOCK DATA FOR Ta WIRE  
REINFORCED TaC COMPOSITES

| Material           | Orientation | Thermal Shock Index     |                         |  |
|--------------------|-------------|-------------------------|-------------------------|--|
|                    |             | For Crack<br>Initiation | For Fracture<br>252/255 |  |
| RVC Graphite       | WG          | —                       | —                       |  |
| 60 vol % Ta wire + | WG          | 80/100                  | can't fracture*         |  |
| 40 vol % TaC       | —           | —                       | —                       |  |
| 60 vol % Ta wire + | AG          | 70/80                   | ~ 225                   |  |
| 40 vol % TaC       | —           | —                       | —                       |  |
| 70 vol % Ta wire + | WG          | 80/100                  | can't fracture*         |  |
| 30 vol % TaC       | —           | —                       | —                       |  |
| 70 vol % Ta wire + | AG          | 60/80                   | ~ 200                   |  |
| 30 vol % TaC       | —           | —                       | —                       |  |

\* Melting of Ta fibers occurs before fracture

Table II  
COMPARISON OF PREDICTED AND  
EXPERIMENTAL VALUES OF THERMAL  
CONDUCTIVITY OF TaC-Ta (WIRE)  
HOT-PRESSED COMPOSITE BODIES (W/cm<sup>2</sup>K at  
33°C)

| P <sub>TaC</sub>                             | P <sub>Ta</sub> | $\rho/\rho_0 = 1$<br>Pre-<br>dicted | $\rho/\rho_0$ | $\rho/\rho_0$<br>Pre-<br>dicted | Experi-<br>mental | 30 |
|----------------------------------------------|-----------------|-------------------------------------|---------------|---------------------------------|-------------------|----|
| 0                                            | 1.0             | 0.576                               | 1.0           | —                               | —                 |    |
| 1.0                                          | 0               | 0.2657                              | 1.0           | —                               | —                 |    |
| AG (parallel to the pressing direction)      |                 |                                     |               |                                 |                   |    |
| 0.90                                         | 0.10            | 0.2890                              | 0.8042        | 0.0838                          | 0.0850            | 35 |
| 0.70                                         | 0.30            | 0.3348                              | 0.8300        | 0.1095                          | 0.1135            |    |
| 0.50                                         | 0.50            | 0.3915                              | 0.8392        | 0.1335                          | 0.1470            |    |
| 0.40                                         | 0.60            | 0.4217                              | 0.8375        | 0.1421                          | 0.1768            |    |
| 0.30                                         | 0.70            | 0.4531                              | 0.8069        | 0.1332                          | 0.200             |    |
| WG (perpendicular to the pressing direction) |                 |                                     |               |                                 |                   |    |
| 0.90                                         | 0.10            | 0.2928                              | 0.8531        | 0.1075                          | 0.0795            | 40 |
| 0.70                                         | 0.30            | 0.3466                              | 0.8480        | 0.1234                          | 0.0935            |    |
| 0.50                                         | 0.50            | 0.4059                              | 0.8232        | 0.1283                          | 0.1140            |    |
| 0.40                                         | 0.60            | 0.4365                              | 0.8434        | 0.1515                          | 0.1628            |    |
| 0.30                                         | 0.70            | 0.4678                              | 0.8125        | 0.1403                          | 0.1845            |    |

Table III shows x-ray diffraction data for various TaC-chopped Ta wire composites. The numbers refer

to the volume percent TaC or Ta. "As pressed" means the composite prepared by hot pressing at 1,800°C for about one-half hour. "Heat treated" means exposed to 2,300°C for 10 hours in a hydrogen environment after being hot pressed. It can be seen that the hot pressed composites show some slight reaction of the Ta fibers with the surrounding TaC matrix to produce the lesser carbide Ta<sub>2</sub>C. The heat treated specimens having higher Ta fiber contents show a much more pronounced reaction between the fibers and the surrounding TaC matrix to produce Ta<sub>2</sub>C. The strong presence of the hydride phase indicates that even after 10 hours at 2,300°C a substantial amount of the Ta remains non-carbided. It is not critical to this invention that the fibers remain substantially present as the metal. The lesser metal carbides have physical and mechanical properties that are sufficiently different than those of the monocarbide matrix that crack propagation is stopped or greatly impeded on reaching them. They thus serve to prevent or greatly inhibit fracturing in substantially the same manner that the metal fibers do.

TABLE III  
X-RAY DIFFRACTION DATA FOR TaC-CHOPPED  
Ta WIRE COMPOSITES

| Sample Description        | Phases Present     |                   |                   |
|---------------------------|--------------------|-------------------|-------------------|
|                           | Strong             | Medium            | Weak              |
| 90 TaC-10 Ta as pressed   | TaC                |                   | Ta <sub>2</sub> C |
| 70 TaC-30 Ta as pressed   | TaC                |                   | Ta <sub>2</sub> C |
| 50 TaC-50 Ta as pressed   | TaC                | Ta <sub>2</sub> C |                   |
| 40 TaC-60 Ta as pressed   | TaC                | Ta <sub>2</sub> C |                   |
| 30 TaC-70 Ta as pressed   | TaC                |                   | Ta <sub>2</sub> C |
| 90 TaC-10 Ta heat-treated | TaC                |                   |                   |
| 70 TaC-30 Ta heat-treated | TaC                |                   |                   |
| 50 TaC-50 Ta heat-treated | Ta <sub>2</sub> C  |                   | Ta <sub>2</sub> C |
| 40 TaC-60 Ta heat-treated | TaH <sub>0.8</sub> |                   | TaC               |
| 30 TaC-70 Ta heat-treated | Ta <sub>2</sub> C  |                   |                   |
|                           | TaC                |                   |                   |
|                           | TaH <sub>0.8</sub> |                   |                   |

What we claim is:

1. A structural material having an improved thermal stress resistance at temperatures in excess of 2,000°C comprising a composite of 50 volume percent TaC and 50 volume percent chopped Ta fibers.

\* \* \* \* \*